

# UNITED STATES PATENT OFFICE.

TRYGVE D. YENSEN, OF SWISSVALE, PENNSYLVANIA.

## MAGNETIC IRON PRODUCT.

1,277,524.

No Drawing.

Specification of Letters Patent.

Patented Sept. 3, 1918.

Application filed June 11, 1917. Serial No. 173,971.

*To all whom it may concern:*

Be it known that I, TRYGVE D. YENSEN, a citizen of the United States, residing at Swissvale, county of Allegheny, State of 5 Pennsylvania, (whose post-office address is 2113 Delaware Ave., Swissvale, Pennsylvania,) have invented certain new and useful Improvements in Magnetic Iron Products, of which the following is a specification.

The present invention relates to iron products having unusual magnetic properties, particularly at high flux densities.

Until a few years ago, pure iron was supposed to have a higher saturation intensity of magnetization than any other material, or in other words, to be the most magnetic material in existence. In 1912, however, Weiss showed that cobalt when alloyed with 15 iron will make the latter even more magnetic than in the pure state. Weiss found that the alloy corresponding to the composition  $Fe_2Co$  has a saturation intensity of magnetization,  $I_s$ , 10% higher than that of the purest iron then in existence, the value  $I_s$  for pure iron being 1750, while that for  $Fe_2Co$  being about 1950. ( $B=4\pi I+H$ , where  $B$ =the total magnetic flux density in 20 gausses,  $H$ =the magnetizing force in gilberts per cm., and  $I$ =the intensity of magnetization which approaches the limit  $I_s$ , when the material is saturated.)

While thus the alloy  $Fe_2Co$  has very desirable characteristics, the cost of cobalt 35 makes the alloy very expensive. By my present invention, I approach the desirable characteristics of the iron-cobalt alloys by means of a substantially pure iron, having the additional advantages over the iron-cobalt alloys of being much more easily worked.

My earlier application for Letters Patent, Serial No. 82340, relates to iron and iron alloys having unusual magnetic properties, 45 my preferred method comprising vacuum fusion in connection with subsequent annealing at temperatures between 900 and 1100° C. For this purpose the product may or may not be pure iron.

The present invention concerns itself more particularly with unusual magnetic properties at exceedingly high inductions and relates only to substantially pure iron. The products may or may not have unusual magnetic properties at low and medium densities.

The products may take the form of rolling mill or bloomery ingots or castings or further products worked therefrom into suitable forms.

To obtain my improved products, I make use of a low carbon iron in which phosphorus, sulfur and manganese have, by well known methods, been reduced to a low figure, preferably to 0.05 per cent. or less, 65 when taken in the aggregate, and containing no appreciable amounts of other elements that can not be eliminated by the subsequent treatment. In my preferred process the iron is further refined by subjecting 70 it, in the molten state, to the action of a vacuum in any suitable manner. The iron may, for example, be melted in a vacuum furnace, or it may be melted under atmospheric pressure and then transferred to a 75 vacuum tank, where suitable means are provided for retaining it in the molten state during the subsequent refining process. This process is to be carried on at such a high temperature, at such a pressure, and 80 for such a length of time (from  $\frac{1}{2}$  to 2 hours, at an absolute pressure of not more than 5 cm. of mercury, and at a bath temperature of at least 1550° C.) that the gases will be substantially eliminated from the 85 bath, and furthermore, that the carbon content of the finished product will be not more than 0.05 per cent. For the best results the carbon content should not be more than 0.01 per cent. The addition of some iron oxid 90 may be necessary for the elimination of the carbon.

After the elimination of the carbon and the gases, the iron is to be further deoxidized, if necessary, to such an extent that 95 the oxygen content of the finished product is 0.05 per cent., or preferably less. The deoxidizing agent used should be of such a character as to accomplish the deoxidation without leaving any appreciable residue in 100 the iron itself or without alloying with the iron. Aluminum may be employed very satisfactorily for this purpose as it does not begin to alloy with the iron until the iron is practically free from oxid.

No alloying elements should be added to the iron, as the purpose of the invention is to obtain a product containing as much pure iron as possible per unit volume, and containing at least 99.70 per cent. Fe.

The refined iron should be allowed to solidify under such conditions as not to be

contaminated by gases or other impurities. Allowing it to solidify *in vacuo* may be necessary for the best results. Finally, any subsequent treatment, whether mechanical or heat treatment, should be done in such a way as to leave the iron practically uncontaminated.

By the herein-described process, it is possible to obtain iron with a saturation intensity 10 of magnetization,  $I_s$ , considerably in excess of 1750, the value for the best grades of iron heretofore known and even exceeding 1800 by a considerable amount. The values of  $I$  at lower flux densities are correspondingly 15 increased by my method.

The method used for obtaining  $I_s$  is that due to Kennelly, which consists in plotting the  $H-\rho$  curve up to  $H=500$  gilberts per 20 cm. or higher, and from the slope of this curve calculate  $I_s$ .

$$\left( \rho = \frac{H}{B} \right).$$

The Isthmus method may also be employed.

Having thus described my invention, what 25 I claim as new and desire to secure by Letters Patent is:

1. An iron product, containing at least 99.70 per cent. iron, characterized by a saturation intensity of magnetization,  $I_s$ , of 1750 30 to 1850.
2. An iron product, containing at least 99.70 per cent. iron, substantially degasified, characterized by a saturation intensity of magnetization,  $I_s$ , of 1750 to 1850. 35
3. An iron product containing at least 99.70 per cent. iron, characterized by a saturation intensity of magnetization,  $I_s$ , of 1800 to 1850.
4. An iron product containing not over 40 0.05 per cent. carbon, in which manganese, phosphorus and sulfur have been reduced to 0.05 per cent. or less, when taken in the aggregate, and oxygen to 0.05 per cent. or less, and containing at least 99.70 per cent. 45 iron, characterized by a saturation intensity of magnetization,  $I_s$ , of 1800 to 1850.

TRYGVE D. YENSEN.